

Sept. 15, 1925.

1,553,976

V. BERNOT ET AL

METHOD OF MANUFACTURING PAPER PULP

Filed Jan. 27, 1921

Fig. 2



Fig. 1



Fig. 3.



Proprietor

Victor Bernot  
Pierre Raymond Fournier

by *A. Blawie and Co*  
Attorneys

## UNITED STATES PATENT OFFICE.

VICTOR BERNOT AND PIERRE RAYMOND FOURNIER, OF BOULOGNE-SUR-SEINE, FRANCE, ASSIGNORS TO SOCIÉTÉ "LA PAILLE INDUSTRIELLE," OF NOYON, FRANCE.

## METHOD OF MANUFACTURING PAPER PULP.

Application filed January 27, 1921. Serial No. 440,470.

*To all whom it may concern:*

Be it known that we, VICTOR BERNOT, a citizen of the Republic of France, and residing at Boulogne-sur-Seine, 14 bis Rue de 5 Sevres, in the Republic of France, and PIERRE RAYMOND FOURNIER, a citizen of the Republic of France, and residing at Boulogne-sur-Seine, 14 bis Rue de Sevres, have invented certain new and useful Improvements in Methods of Manufacturing Paper Pulp, of which the following is a specification.

This invention relates to a method and apparatus for the manufacture of paper pulp.

15 The current method of manufacture of paper pulp comprises a series of successive operations such as sorting the raw material in the shape of natural or artificial vegetable fabrics, washing or dust removal, cutting up, lye treatment, washing after the same, separation of fibres, bleaching and subsequent washing. The most important of these operations are the lye treatment and the separation of fibre. The first of 20 these operations serves to dissolve as much as possible the foreign bodies which surround and connect the fibres of pure cellulose, and is usually carried out in a digester at a pressure of about 3 kilogrammes per 25 square centimeter, the operation lasting from 2 to 8 hours, or often more. After washing for 1 to 4 hours in a washing apparatus, the lye-treated material is submitted to a fibre separating process, for the 30 purpose of separating the fibres which are still collected in larger or smaller masses. This mechanical operation is generally carried out in a drum containing fixed and moving blades. The paper pulp which is 35 thus obtained is only in the partially finished condition, inasmuch as it is not homogeneous and requires to be refined in order to be used for the manufacture of high grade papers.

40 The process of manufacture as thus carried out requires successive treatments of the material, and cannot be considered as a continuous process. It requires a considerable amount of labor and complicated and 45 cumbersome apparatus, while the successive chemical and mechanical operations are of long duration, the yield being only moderate owing to the fact that the long duration of the chemical operations has a ten-

dency to cause the partial hydrolysis of the 55 fibres. Moreover, the mechanical treatment of the non-homogeneous substances has an unduly energetic and prejudicial action upon the fibres which are already separated but as an insufficient effect upon the aggregates of fibres which have not been sufficiently separated by the lye treatment.

In our invention these inconveniences are obviated. According to this invention, a 60 continuous process is employed whereby the material is continuously introduced, lye-treated, and has the fibres thereof separated in a continuous current of lye bath. The 65 separate fibres which are carried along by this current are filtered out and removed 70 from the filter either in a continuous manner or at more or less frequent intervals, whereas the lye bath is preferably returned to the point at which the continuous feeding 75 of the material is effected. The mechanical treatment of the aggregates of fibres is thus carried out in the presence of the lye bath at the same time as the adherent substances are dissolved or rendered soluble, and the 80 separate fibres are submitted to the contact with the lye and the mechanical action of the fibre-separating members for the shortest possible time.

Important advantages will result therefrom which will be hereinafter set forth.

85 The accompanying drawings which are given by way of example show a diagrammatic view of a series of apparatus wherein the present process is applied.

Figure 1 is a diagrammatic view of the 90 whole series of apparatus.

Figure 2 is a longitudinal section of a lye-treating apparatus and a fibre-separating apparatus suitably combined.

Figure 3 is an elevational view of one of 95 the perforated plates.

The lye-treating apparatus comprises a horizontal cylinder 1 whereon is disposed a feed hopper 2 employed for the continuous feeding of the vegetable matter to be treated by the lye-bath. The said cylinder contains a shaft 3 having formed or secured thereon a screw conveyor 4 for propelling the material under treatment from the end adjacent the feeding hopper to the opposite end of the device. A portion of the said screw-member is preferably 100 adapted to cooperate with the internal edge 105

of the feeding aperture which acts as a cutting blade in order to cut up the raw material into large fragments upon the introduction of the same into the cylinder.

5 Within a recess 5 provided in the wall of the cylinder is disposed a member 6 in the form of a wheel which is loosely rotatable upon the shaft thereof 7 and engages the threads of the screw member 4. The said 10 wheel serves to prevent the free movement of the material about the said screw member which might take place in spite of the fluid nature thereof, and the material is now obliged to move forward as the screw 15 rotates. The said cylinder which is chiefly used for the lye treatment, is heated, if required by a furnace of any suitable disposition 8, or by like heating devices.

The size of the cylinder as well as the 20 pitch and rate of rotation of the screw may be varied according to the character of the substance under treatment, these factors being so determined as to afford the proper duration for the movement of the material 25 whereby the latter shall be sufficiently penetrated by the lye bath upon attaining the end of the cylinder 1.

For all the material under operation, wood excepted, the duration of the lye 30 treatment does not usually exceed 30 minutes. The matter which arrives at the end 9 of the cylinder still retains substantially the same shape as it had at the feeding end, and the separation of the material is carried out chiefly in the fibre-separating apparatus. It may however be advantageous 35 to dispose adjacent the perforated end 9 of the cylinder 1 a rotary knife 10 for a rough cutting up of the fibrous matter, the 40 said knife cooperating with the bottom part 9 somewhat after the manner of the knife member and perforated plate of the current type of meat cutter.

The fibre-separating apparatus comprises 45 a cylinder 11 preferably disposed in alignment with the lye-treating cylinder and having therein a series of stationary partitions 12<sup>a</sup>, 12<sup>b</sup>, 12<sup>c</sup> etc. forming various chambers, 10 for instance, such as 13<sup>a</sup>, 13<sup>b</sup>, 13<sup>c</sup> etc. the 50 said partitions being provided with the apertures 14<sup>a</sup>, 14<sup>b</sup> etc. of decreasing width, the apertures 14<sup>a</sup> having for instance several centimeters width whereas the apertures 14<sup>c</sup> are reduced to very narrow slits 55 for the purpose of allowing only the individual fibres to pass through. Within the said chambers are disposed the rotary stirring members 15<sup>a</sup>, 15<sup>b</sup> . . . 15<sup>k</sup> which are secured to the shaft 16 disposed according to 60 the axis of the cylinder 11. The said shaft is situated preferably within the shaft 3, this latter being made hollow to this effect, and it also carries the rotary knife 10. A 65 small space, for instance 2 millimeters, is preferably provided between the partitions

12 and the stirring members 15 to prevent the shearing of the fibres and to cause the latter to be separated from each other by the effect of easy friction within the body of the lye bath and without rough handling. 70

The shafts 3 and 16 are actuated for instance by belting disposed upon the pulleys 17 and 18 or by gearing or the like, in such manner as to effect the rotation of the stirring members 15 at a much higher speed 75 than that of the screw 4, whereby the forward movement of the lye bath and the material shall be much slower than that of the stirring or fibre-separating members. As the material in the chambers 13<sup>a</sup>, 13<sup>b</sup> 80 etc. becomes separated into fibrous aggregates which are sufficiently fine to pass through the apertures of the following partition, these aggregates will pass into the following chamber, being drawn along by 85 the current, of the lye bath, and so on, until they are finally reduced to the state of separate fibres which are alone able to pass out through the slits of the partition 12<sup>k</sup>. It is obvious that the fibres which are more 90 readily separated will pass off more quickly than the fibres which adhere closely together, and each class of fibres is caused to remain in the separating apparatus only for 95 the time which is strictly necessary to produce the separating action.

Upon leaving the fibre-separating cylinder, the paste drops into one or more filter presses 19 of any suitable construction 100 whereby the cellulose fibres are retained and separated from the lye bath. It should be remarked that in the present apparatus the lye is not submitted to a high pressure as in the usual digesters. The lye bath which is discharged from the filter press or presses 105 is conducted through the piping 20 to a pump 21 or other elevating device which returns the same to the hopper 2. The fibres remaining in the filtering devices are discharged therefrom at more or less frequent 110 intervals or by a continuous process, according to the character of the apparatus employed, and the fibres are then ready for the washing process. After a sufficient washing, they constitute a pulp which is suitable 115 for paper manufacture.

The present method affords various advantages as compared with known methods, which may be set forth as follows:

A single chemical and mechanical operation is substituted for the two different operations of lye treatment and fibre separation. 120

The production of clean and separated fibres, representing paper paste, is now carried out in a continuous manner, this affording a very considerable advantage as concerns cost of operation. 125

The apparatus takes up but a small space 130 and requires a minimum of hand labor.

The lye bath is used in a systematic and complete manner, resulting in a minimum cost of lye substances.

Inasmuch as the fibres are discharged as soon as separated, they are not submitted to an unduly prolonged action of lye baths, and they have no tendency to become hydrolyzed.

The separation of the fibrous aggregates in suspension in the liquid is effected without rough handling and without useless deterioration of the fibres.

The herein described combined chemical and mechanical action is so effective that the same apparatus may be used for the treatment of the greater part of natural or artificial vegetable substances with equal facility, and textile products containing oily substances, such as greasy waste, can be directly transformed into paper paste without any previous washing.

The quantity of material under treatment at any given moment is relatively small, whence it follows that a large or small amount of substance may be treated with equal facility and with the same relative economy, and a great variety of substances can be treated successively without requiring any stoppage or cleaning of the apparatus, whereby paper paste of various qual-

ities may be produced in a continuous manner.

Inasmuch as the fibre separation is obtained with the minimum amount of lye bath, the fibres will not show a tendency to agglomerate into small masses, and moreover, in case a hot treatment is to be carried out, the loss of heat will be a minimum by reason of the fact that only a small quantity of material is placed under treatment.

Claim:

A process for the manufacture of paper paste in an endless current of suitable liquid, wherein the raw fibrous substances are introduced in a continuous manner at a given point of the said current and are caused to pass through the fibre-removing elements after having been saturated with the said liquid, the fibres being removed from the current at a second point in the stream of liquid in the form of a pulp which is ready for use, whereby the liquid does not pass again through the same points before all the fibres are removed.

In testimony that we claim the foregoing as our invention, we have signed our names.

VICTOR BERNOT.

PIERRE RAYMOND FOURNIER.